

## UNITED STATES PATENT OFFICE

HUGO BEINROTH, OF HAMBURG, GERMANY, ASSIGNOR TO HEYDEN CHEMICAL CORPORATION, OF NEW YORK, N. Y., A CORPORATION OF NEW YORK

## METHOD OF APPLYING SIGNS TO GLASS

No Drawing. Application filed March 23, 1928, Serial No. 264,281, and in Germany March 29, 1927.

This invention relates to the production of signs and it particularly relates to the production of signs on glass, for instance on the back of show-windows and the like glass panes.

The production of signs, figures, or the like, from materials having a metallic luster, or being colored, especially the production of firm names or similar signs in gold or 10 silver on the inner side of a show window, always entailed a rather cumbersome and costly procedure. In order to obtain durable signs, or figures, in gold or silver, one had to resort to films of the genuine precious 15 metals. Inasmuch as such metals could only be produced in films of small dimensions, lettering windows and similar work was always slow. Moreover, the high luster of the films of precious metals proved not mellow enough 20 to yield easily legible signs. It was necessary therefore, in the most cases, to prepare the surface of the glass first by either slightly etching it or give it a coat of lacquer or varnish, or eventually deaden slightly the luster 25 of the precious metal by suitable means.

I have now found a process by which the application of films of the precious metals is avoided. In the operation of my invention I apply only films made of ordinary 30 bronze powder. It is important that the bronze particles are embedded in a binding material in which they are hermetically sealed; such binding materials are for instance cellulose esters, such as nitro-cellulose, 35 acetyl-cellulose, formyl-cellulose, and the like esters, cellulose-ether, gelatine or any other, preferably transparent, colorless material forming films. The films may be used with or without paper backing. Instead of 40 a film proper I may also use paper, tissues or any other similar texture coated with a layer of bronze or color. I apply for instance thin bronze tissue paper, or colored pargamyn paper, such as used in some countries for finishing the mouth pieces of cigarettees.

Remarkably well suited for the purposes of my invention are the rolls of films as obtained by the process of von Hoessle & Richter, described in U. S. Patent No.

1,707,828, issued on April 2, 1929. Though even the very fine films obtained by this process do not cling quite as readily to glass as for instance precious metal films, suitable adhesives, for instance such as gelatine, 55 damar-varnish, or the like, cause it to stick firmly to glass. It is particularly advantageous that that part of the window, which is to be lettered, can be covered with a single big sheet of bronze film and that it is not necessary to align one small slip after the other. The rolls of bronze films made by the von Hoessle-Richter process can be furnished in any length and widths up to 28 inches.

To produce for instance a window sign of 60 28 inches height and 80 inches length, it is only necessary to affix a film of slightly more than the above dimensions by means of a solution of gelatine to the inner side of the window, which of course was previously 65 properly cleaned. The gelatine solution, which I found very suitable for this purpose, contained 8 sheets of gelatine in a liter of water. The bronze film is then pressed upon the glass with blotting paper and a squeegee 70 roller and as much of the gelatine solution is pressed out from between the glass and the film as can safely be done in view of the fragility of the window pane. By working in this manner the film adheres perfectly 75 smoothly to the glass, especially the more the drying proceeds. The drying can also be accelerated by artificial heat, for instance by means of a fan blowing heated air upon the film. Though the desired sign in reversed 80 position can be entered directly upon the bronze surface, and the superfluous parts of the film can be erased, the process described below is more advantageous.

In this process I proceed exactly as described above until the bronze film has dried and at that stage I coat then the film with a solution of damar varnish and turpentine and allow then the solvent to evaporate for some minutes until the varnish becomes 85 sticky. Then I apply a covering material which will admit of cutting out the letters with well defined edges. Among other materials I found that tin foil answers this purpose especially well. I trace then the let- 90 95 100

ters in reversed position upon this tin foil and then cut them out with a sharp knife, taking care that the edges present a clean cut. The knife must cut through to the glass so as to have also the bronze film cut through.

5. Thereupon all these parts of the covering or protecting material are ripped off which do not form a part of the desired sign.

Whenever, as in the present case, for the 10 application of the bronze film upon the glass an adhesive was used which like gelatine, does not adhere so strongly as the damar varnish used for the cover, or tin foil, the superfluous parts of the bronze film are also torn off so that only the letters remain which are pressed once more with the squeegee roller. Should any spots of varnish show on the 15 glass, then I remove the same with turpentine and similarly I remove with luke-warm 20 water the gelatine sticking on the glass between the letters. These letters are thereupon pressed again and are then finally covered with a layer of lacquer or varnish, or of suitable paint. The letters can also be 25 provided with a rim of varnish or lacquer so as to show off more distinctly. In case it is desired to have a sign show off from a dark ground then two or three coats of varnish, stained with the desired color, are 30 applied over the whole part of the glass, including the letters; by this contrast any letters, figures, or decorations are then distinctly visible. Or if desired, a silver or mercury foil can be applied upon the glass, extending also over the sign, and one obtains 35 then a mirror from which the golden, or colored letters show off well. It is of course understood that instead of bronze films such of the precious metals, gold, silver, etc. may 40 be used for the signs, that by the addition of dyestuffs or by the application of colored bronzes a great variation of color effects may be produced, or that films made with any desired pigment may be used.

45. The procedure for the manufacture of glass letters is similar as described above. I coat then such letters for instance on their back with damar varnish, allow the same to dry until it becomes sticky, apply then the thin 50 bronze film and rub the same thereafter with a soft piece of cloth from the middle to the edges. Thereupon I coat the surface repeatedly with damar varnish and finally provide it with a protective coat, for instance tin foil. 55. As a finishing touch I cut off all parts projecting beyond the edges of the letters. Colored letters are similarly produced.

What I claim is:

1. The method of applying signs on the 60 rear side of glass, consisting in applying an adhesive to the glass, pressing tightly upon the glass a strip of a film, having a coloring matter embedded therein, providing then a coat of another adhesive on said film, im- 65 pressing a thin foil of an easily cut protec-

tive material upon the adhesive when highly sticky, imprinting the reversed sign upon the aforesaid foil, cutting the layers through to the glass along the edges of the sign, and ripping off the superfluous parts of the layers when dry. 70

2. The method of applying signs on the rear side of the glass, consisting in applying an adhesive to the glass, pressing tightly upon the glass a strip of a film of a transparent, colorless material, larger in size than the sign and having a coloring matter embedded therein, providing then a coat of another adhesive on said film, impressing a thin foil of an easily cut protective material upon the adhesive when highly sticky, imprinting the reversed sign upon the aforesaid foil, cutting the layers through to the glass along the edges of the sign, and ripping off the superfluous parts of the layers when dry. 75

3. The method of applying signs to the rear side of glass, consisting in applying an adhesive of moderate power to the glass, pressing tightly upon the glass a strip of a film of a transparent, colorless substance, larger in size than the sign and having a coloring matter embedded therein providing on top of the aforesaid film a coat of an adhesive of stronger power than that below the 80 said film, impressing a thin foil of an easily cut protective material upon the stronger adhesive, imprinting the reversed sign upon the aforesaid foil, cutting the layers through to the glass along the edges of the sign, and ripping off the superfluous parts of layers when dry. 85

4. The method of applying signs to the rear side of glass, consisting in applying a solution of gelatine to the surface of the glass, pressing tightly upon the glass a strip of a film of a transparent colorless substance, larger in size and having a metal bronze embedded therein, providing on top of said film a coat of damar varnish, impressing a film of tin foil upon said damar varnish when highly sticky, imprinting the reversed sign upon the tin foil, cutting the layers through to the glass along the edges of the sign, and ripping off the superfluous parts of the layers when dry. 90

In witness whereof I have hereunto set my hand this 8th day of March, 1928.

HUGO BEINROTH.

120

125

130